



US006162549A

# United States Patent [19]

Camp et al.

[11] Patent Number: 6,162,549

[45] Date of Patent: Dec. 19, 2000

[54] **DAY/NIGHT IMAGING DISPLAY MATERIAL WITH BIAXIALLY ORIENTED POLYOLEFIN SHEET**

[75] Inventors: **Alphonse D. Camp**, Rochester; **Peter T. Aylward**, Hilton; **Robert P. Bourdelais**, Pittsford, all of N.Y.

[73] Assignee: **Eastman Kodak Company**, Rochester, N.Y.

[21] Appl. No.: 09/156,061

[22] Filed: Sep. 17, 1998

[51] Int. Cl.<sup>7</sup> ..... B41M 5/00

[52] U.S. Cl. ..... 428/523; 428/195; 428/304.4; 428/516

[58] Field of Search ..... 8/471; 428/195, 428/913, 914, 304.4, 910, 516, 523; 503/227

## [56] References Cited

### U.S. PATENT DOCUMENTS

|           |         |                |
|-----------|---------|----------------|
| 3,944,699 | 3/1976  | Mathews et al. |
| 4,187,113 | 2/1980  | Mathews et al. |
| 4,283,486 | 8/1981  | Aono et al.    |
| 4,632,869 | 12/1986 | Park et al.    |
| 4,758,462 | 7/1988  | Park et al.    |

|           |         |                               |
|-----------|---------|-------------------------------|
| 4,900,654 | 2/1990  | Pollock et al. .              |
| 4,912,333 | 3/1990  | Roberts et al. .              |
| 4,977,070 | 12/1990 | Winslow .                     |
| 5,055,371 | 10/1991 | Lee et al. .                  |
| 5,100,862 | 3/1992  | Harrison et al. .             |
| 5,212,053 | 5/1993  | McSweeney et al. .            |
| 5,244,861 | 9/1993  | Campbell et al. .             |
| 5,314,861 | 5/1994  | Morohoshi et al. .... 503/227 |
| 5,387,501 | 2/1995  | Yajima et al. .               |
| 5,389,422 | 2/1995  | Okazaki et al. .              |
| 5,466,519 | 11/1995 | Shirakura et al. .            |

### FOREIGN PATENT DOCUMENTS

0 662 633 A1 12/1995 European Pat. Off. .  
WO 94/04961 3/1994 WIPO .

Primary Examiner—Bruce H. Hess  
Attorney, Agent, or Firm—Paul A. Leipold

## [57] ABSTRACT

The invention relates to an imaging element comprising a transparent polymer sheet, at least one layer of biaxially oriented polyolefin sheet and at least one image receiving layer wherein said polymer sheet has a stiffness of between 20 and 100 millinewtons, and said biaxially oriented polyolefin sheet has a spectral transmission of between 35% and 90% and a reflection density of between 15% and 65%.

**38 Claims, No Drawings**

**DAY/NIGHT IMAGING DISPLAY MATERIAL  
WITH BIAXIALLY ORIENTED POLYOLEFIN  
SHEET**

**FIELD OF THE INVENTION**

This invention relates to imaging materials. In a preferred form it relates to base materials for reflective and transmission display.

**BACKGROUND OF THE INVENTION**

It is known in the art that imaging display materials are utilized for advertising, as well as decorative displays of images. Since these display materials are used in advertising, the image quality of the display material is critical in expressing the quality message of the product or service being advertised. Further, a display image needs to be high impact, as it attempts to draw consumer attention to the display material and the desired message being conveyed. Typical applications for display material include product and service advertising in public places such as airports, buses and sports stadiums, movie posters, and fine art photography. The desired attributes of a quality, high impact display material are a slight blue density minimum, durability, sharpness, and flatness. Cost is also important, as photographic display materials tend to be expensive as the imaging process is equipment intensive and requires processing chemicals. For imaging display materials, traditional paper bases are undesirable, as they suffer from a lack of durability for the handling and captured display of large format images. The use display materials such as lithographic prints or ink jet prints could be expanded if image quality was improved.

In the formation of color paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult requiring great care and expense to ensure proper laydown and cooling of the polyethylene layers. The formation of a suitably smooth surface would also improve image quality, as the display material would have more apparent blackness as the reflective properties of the improved base are more specular than the prior materials. As the whites are whiter and the blacks are blacker, there is more range in between and, therefore, contrast is enhanced. It would be desirable if a more reliable and improved surface could be formed at less expense.

Prior art photographic reflective papers comprise a melt extruded polyethylene layer which also serves as a carrier layer for optical brightener and other whitener materials, as well as tint materials. It would be desirable if the optical brightener, whitener materials, and tints, rather than being dispersed could be in single melt extruded layer of polyethylene, could be concentrated nearer the surface where they would be more effective optically.

Prior art photographic display materials historically have been classified as either reflective or transmission. Reflective display materials typically are highly pigmented image supports with a light sensitive silver halide coating applied. Reflective display materials are typically used in commercial applications where an image is used to convey an idea or message. An application example of a reflective display material is product advertisement in a public area. Prior art reflective display materials have been optimized to provide a pleasing image using reflective light. Transmission display materials are used in commercial imaging applications and

are typically backlit with a light source. Transmission display materials are typically a clear support with an incorporated diffuser coated with a light sensitive silver halide emulsion. Prior art transmission display materials have been optimized to provide a pleasing image when the image is backlit with a variety of light sources. Because prior art reflective and transmission products have been optimized to be either a reflection display image or a transmission display image, two separate product designs must exist in manufacturing and two inventories of display materials must be maintained at the commercial printer. Further, when the quality of the backlighting for transmission display material is reduced when, for example, a backlight burns out or the output of the backlight decreases with the age, the transmission image will appear dark and reduce the commercial value of the image. It would be desirable if an image support could function both as a reflection and transmission display material.

Prior art transmission display materials use a high coverage of light sensitive silver halide emulsion to increase the density of the image compared to photographic reflective print materials. While increasing the coverage does increase the density of the image in transmission space, the time to image development is also increased as the coverage increases. Typically, a high density transmission display material has a developer time of 110 seconds compared to a developer time of 45 seconds or less for photographic print materials. Prior art high density transmission display materials, when processed, reduce the productivity of the development lab. Further, coating a high coverage of emulsion requires additional drying of the emulsion in manufacturing reducing the productivity of emulsion coating machines. It would be desirable if a transmission display material was high in density and had a developer time less than 50 seconds.

Prior art reflective photographic materials with a polyester base use a  $TiO_2$  pigmented polyester base onto which light sensitive silver halide emulsions are coated. It has been proposed in WO 94/04961 to use an opaque polyester containing 10% to 25%  $TiO_2$  for a photographic support. The  $TiO_2$  in the polyester gives the reflective display materials an undesirable opalescent appearance. The  $TiO_2$  pigmented polyester also is expensive because the  $TiO_2$  must be dispersed into the entire thickness, typically from 100 to 180  $\mu m$ . The  $TiO_2$  also gives the polyester support a slight yellow tint which is undesirable for a photographic display material. For use as a photographic display material, the polyester support containing  $TiO_2$  must be tinted blue to offset the yellow tint of the polyester causing a loss in desirable whiteness and adding cost to the display material. It would be desirable if a reflective display support did not contain any  $TiO_2$  in the base and could be concentrated near the imaging forming layers.

Prior art photographic transmission display materials, while providing excellent image quality, tend to be expensive when compared with other quality imaging technologies such as ink jet imaging, thermal dye transfer imaging, and gravure printing. Since photographic transmission display materials require an additional imaging processing step compared to alternate quality imaging systems, the cost of a transmission photographic display can be higher than other quality imaging systems. The processing equipment investment required to process photographic transmission display materials also requires consumers to typically interface with a commercial processing lab increasing time to image. It would be desirable if a high quality transmission display support could utilize nonphotographic quality imaging technologies.

Photographic reflection/transmission display materials have considerable consumer appeal, as they allow images to be printed on high quality support for home or small business use. Consumer use of photographic display materials generally has been cost prohibitive since consumers typically do not have the required volume to justify the use of such materials. It would be desirable if a high quality reflection/transmission display material could be used in the home without a significant investment in equipment to print the image.

Prior art photographic display materials use polyester as a base for the support. Typically the polyester support is from 150 to 250  $\mu\text{m}$  thick to provide the required stiffness. A thinner base material would be lower in cost and allow for roll handling efficiency as the rolls would weigh less and be smaller in diameter. It would be desirable to use a base material that had the required stiffness but was thinner to reduce cost and improve roll handling efficiency.

#### PROBLEM TO BE SOLVED BY THE INVENTION

There is a continuing need for an improved product that will present a bright reflective image when viewed directly and also provide a sharp bright image when backlit.

#### SUMMARY OF THE INVENTION

It is an object of the invention to overcome disadvantages of prior display materials.

It is another object to provide a superior, lower cost, and stronger display material.

It is a further object to provide a product that may be provided with an image on each side.

It is another object to provide a day/night display material that utilizes nonphotographic imaging technology.

These and other objects of the invention are accomplished by an imaging element comprising a transparent polymer sheet, at least one layer of biaxially oriented polyolefin sheet and at least one image receiving layer wherein said polymer sheet has a stiffness of between 20 and 100 millinewtons, and said biaxially oriented polyolefin sheet has a spectral transmission of between 35% and 90% and a reflection density of between 15% and 65%.

#### ADVANTAGEOUS EFFECT OF THE INVENTION

The invention provides a material that will when imaged will result in a bright sharp reflective image, as well as allowing for backlighting of the image to also result in a clear sharp image in low light situations.

#### DETAILED DESCRIPTION OF THE INVENTION

The invention has numerous advantages over prior practices in the art. The invention provides a stronger material as the biaxially oriented polyolefin sheet provides flexural rigidity. The material of the invention is lower in cost as a thinner polyethylene terephthalate sheet may be utilized as strength is provided by the biaxially oriented polyolefin sheet. The display material of the invention can be used in the home as digital printing technology such as ink jet printing can be used to apply a high quality image to the support. The time to image is less than a traditional photographic system, as small jobs can be quickly printed as they avoid additional processing steps required by photographic

systems. The material of the invention provides a transmission/reflection display material allowing for a wider range of applications utilizing just one material. Because nonphotographic imaging systems are used to image the support, the display materials are more assessable to the consumer as digital printing systems such as ink jet or thermal dye transfer are widely available and low in cost for small volume. Finally, since the imaging technology used in this invention does not require wet chemistry processing of images, the environmental problems associated with the use and disposal of processing chemicals are avoided. These and other advantages will be apparent from the detailed description below.

The terms as used herein, "top", "upper", "imaging side", and "face" mean the side or toward the side of the laminated support that carries the biaxially oriented sheet. The terms "bottom", "lower side", and "back" mean the side or toward the side of the laminated support opposite of the biaxially oriented sheet. The term as used herein, "transparent" means the ability to pass radiation without significant deviation or absorption. For this invention, "transparent" material is defined as a material that has a spectral transmission greater than 90%. For a photographic element, spectral transmission is the ratio of the transmitted power to the incident power and is expressed as a percentage as follows:  $T_{RGB}=10^{-D/100}$  where D is the average of the red, green, and blue Status A transmission density response measured by an X-Rite model 310 (or comparable) photographic transmission densitometer.

The layers of the biaxially oriented polyolefin sheet of this invention have levels of voiding,  $\text{TiO}_2$  and colorants adjusted to provide optimum reflection and transmission properties. The biaxially oriented polyolefin sheet is laminated to a transparent polymer base for stiffness and for efficient image processing, as well as product handling and display. An important aspect of this invention is that the imaging support is preferably coated with an imaging layer on the top side and the bottom side. These duplitized imaging layers, combined with the optical properties of the biaxially oriented sheet, provide an improved imaging display material that can be used in both reflection and transmission. In reflection, the support of this invention does not allow the imaging on the backside to show through. In transmission, the imaging on the backside gives the image enough density to appear high quality. Without the image on the backside, the display material of this invention would not have enough dye density to appear high quality. The "dual" display material of this invention has significant commercial value in that prior art display materials function as either a reflective display or a transmission display. The display material of this invention can function as both a transmission display and a reflection display.

Further, the thin skin layer on the top of the biaxially oriented polyolefin sheet of this invention can be optimized for image receiving layer adhesion. A thin layer of biaxially oriented polycarbonate allows a solvent based polycarbonate dye receiver layer, typical of thermal dye transfer imaging, to adhere to the base without an expensive primer coating.

Another important aspect of this invention is that using digital, low cost printing technology significantly reduces the time to image compared with a photographic display. Further, the nonphotographic imaging technologies avoid the need for expensive photo processing equipment that is required to process photographic images. The nonphotographic imaging systems also allow home use of the display material of this invention as ink jet printers, for example, are widely available in the home and in offices.

Any suitable biaxially oriented polyolefin sheet may be utilized for the sheet on the top side of the laminated base of the invention. Microvoided composite biaxially oriented sheets are preferred because the voids provide opacity without the use of  $TiO_2$ . Microvoided composite oriented sheets are conveniently manufactured by coextrusion of the core and surface layers, followed by biaxial orientation, whereby voids are formed around void-initiating material contained in the core layer. Such composite sheets are disclosed in, for example, U.S. Pat. Nos. 4,377,616; 4,758,462; and 4,632,869.

The core of the preferred composite sheet should be from 15 to 95% of the total thickness of the sheet, preferably from 30 to 85% of the total thickness. The nonvoided skin(s) should thus be from 5 to 85% of the sheet, preferably from 15 to 70% of the thickness.

The density (specific gravity) of the composite sheet, expressed in terms of "percent of solid density" is calculated as follows:

$$\frac{\text{Composite Sheet Density}}{\text{Polymer Density}} \times 100 = \% \text{ of Solid Density}$$

should be between 45% and 100%, preferably between 67% and 100%. As the percent solid density becomes less than 67%, the composite sheet becomes less manufacturable due to a drop in tensile strength and it becomes more susceptible to physical damage.

The total thickness of the composite sheet can range from 12 to 100  $\mu\text{m}$ , preferably from 20 to 70  $\mu\text{m}$ . Below 20  $\mu\text{m}$ , the microvoided sheets may not be thick enough to minimize any inherent nonplanarity in the support and would be more difficult to manufacture. At thickness higher than 70  $\mu\text{m}$ , little improvement in either surface smoothness or mechanical properties is seen, and so there is little justification for the further increase in cost for extra materials.

"Void" is used herein to mean devoid of added solid and liquid matter, although it is likely the "voids" contain gas. The void-initiating particles which remain in the finished packaging sheet core should be from 0.1 to 10  $\mu\text{m}$  in diameter, preferably round in shape, to produce voids of the desired shape and size. The size of the void is also dependent on the degree of orientation in the machine and transverse directions. Ideally, the void would assume a shape which is defined by two opposed and edge contacting concave disks. In other words, the voids tend to have a lens-like or biconvex shape. The voids are oriented so that the two major dimensions are aligned with the machine and transverse directions of the sheet. The Z-direction axis is a minor dimension and is roughly the size of the cross diameter of the voiding particle. The voids generally tend to be closed cells, and thus there is virtually no path open from one side of the voided-core to the other side through which gas or liquid can traverse.

The void-initiating material may be selected from a variety of materials, and should be present in an amount of about 5-50% by weight based on the weight of the core matrix polymer. Preferably, the void-initiating material comprises a polymeric material. When a polymeric material is used, it may be a polymer that can be melt-mixed with the polymer from which the core matrix is made and be able to form dispersed spherical particles as the suspension is cooled down. Examples of this would include nylon dispersed in polypropylene, polybutylene terephthalate in polypropylene, or polypropylene dispersed in polyethylene terephthalate. If the polymer is preshaped and blended into the matrix polymer, the important characteristic is the size

and shape of the particles. Spheres are preferred, and they can be hollow or solid. These spheres may be made from cross-linked polymers which are members selected from the group consisting of an alkenyl aromatic compound having the general formula  $Ar—C(R)=CH_2$ , wherein Ar represents an aromatic hydrocarbon radical, or an aromatic halohydrocarbon radical of the benzene series and R is hydrogen or the methyl radical; acrylate-type monomers include monomers of the formula  $CH_2=C(R')—C(O)(OR)$  wherein R is selected from the group consisting of hydrogen and an alkyl radical containing from about 1 to 12 carbon atoms and R' is selected from the group consisting of hydrogen and methyl; copolymers of vinyl chloride and vinylidene chloride, acrylonitrile and vinyl chloride, vinyl bromide, vinyl esters having formula  $CH_2=CH(O)COR$ , wherein R is an alkyl radical containing from 2 to 18 carbon atoms; acrylic acid, methacrylic acid, itaconic acid, citraconic acid, maleic acid, fumaric acid, oleic acid, vinylbenzoic acid; the synthetic polyester resins which are prepared by reacting terephthalic acid and dialkyl terephthalates or ester-forming derivatives thereof, with a glycol of the series  $HO(CH_2)_nOH$  wherein n is a whole number within the range of 2-10 and having reactive olefinic linkages within the polymer molecule, the above-described polyesters which include copolymerized therein up to 20 percent by weight of a second acid or ester thereof having reactive olefinic unsaturation and mixtures thereof, and a cross-linking agent selected from the group consisting of divinylbenzene, diethylene glycol dimethacrylate, diallyl fumarate, diallyl phthalate and mixtures thereof.

Examples of typical monomers for making the cross-linked polymer include styrene, butyl acrylate, acrylamide, acrylonitrile, methyl methacrylate, ethylene glycol dimethacrylate, vinyl pyridine, vinyl acetate, methyl acrylate, vinylbenzyl chloride, vinylidene chloride, acrylic acid, divinylbenzene, acrylamidomethylpropane sulfonic acid, vinyl toluene, etc. Preferably, the cross-linked polymer is polystyrene or poly(methyl methacrylate). Most preferably, it is polystyrene and the cross-linking agent is divinylbenzene.

Processes well known in the art yield nonuniformly sized particles, characterized by broad particle size distributions. The resulting beads can be classified by screening the beads spanning the range of the original distribution of sizes. Other processes such as suspension polymerization, limited coalescence, directly yield very uniformly sized particles.

The void-initiating materials may be coated with agents to facilitate voiding. Suitable agents or lubricants include colloidal silica, colloidal alumina, and metal oxides such as tin oxide and aluminum oxide. The preferred agents are colloidal silica and alumina, most preferably, silica. The cross-linked polymer having a coating of an agent may be prepared by procedures well known in the art. For example, conventional suspension polymerization processes wherein the agent is added to the suspension is preferred. As the agent, colloidal silica is preferred.

The void-initiating particles can also be inorganic spheres, including solid or hollow glass spheres, metal or ceramic beads or inorganic particles such as clay, talc, barium sulfate, and calcium carbonate. The important thing is that the material does not chemically react with the core matrix polymer to cause one or more of the following problems: (a) alteration of the crystallization kinetics of the matrix polymer, making it difficult to orient, (b) destruction of the core matrix polymer, (c) destruction of the void-initiating particles, (d) adhesion of the void-initiating particles to the matrix polymer, or (e) generation of undesirable reaction products, such as toxic or high color moieties.

For the biaxially oriented sheets on the top side, suitable classes of thermoplastic polymers for the biaxially oriented sheet and the core matrix-polymer of the preferred composite sheet comprise polyolefins. Suitable polyolefins include polypropylene, polyethylene, polymethylpentene, polystyrene, polybutylene, and mixtures thereof. Polyolefin copolymers, including copolymers of propylene and ethylene such as hexene, butene, and octene are also useful. Polypropylene is preferred, as it is low in cost and has desirable strength properties.

The nonvoided skin layers of the composite sheet can be made of the same polymeric materials as listed above for the core matrix. The composite sheet can be made with skin(s) of the same polymeric material as the core matrix, or it can be made with skin(s) of different polymeric composition than the core matrix. For compatibility, an auxiliary layer can be used to promote adhesion of the skin layer to the core.

The total thickness of the topmost skin layer or top layer of the biaxially oriented polymer sheet should be between 0.20  $\mu\text{m}$  and 1.5  $\mu\text{m}$ , preferably between 0.5 and 1.0  $\mu\text{m}$ . Below 0.5  $\mu\text{m}$  any inherent nonplanarity in the coextruded skin layer may result in unacceptable color variation. At skin thickness greater than 1.0  $\mu\text{m}$ , there is a reduction in the image optical properties such as image resolution. At thickness greater than 1.0  $\mu\text{m}$  there is also a greater material volume to filter for contamination such as clumps, poor color pigment dispersion, or contamination. Low density polyethylene with a density of 0.88 to 0.94 g/cc is a preferred material for the top skin because gelatin based image receiving layers adhere well to low density polyethylene compared to other materials such as polypropylene and high density polyethylene.

Addenda may be added to the topmost skin layer to change the color of the imaging element. For imaging use, a white base with a slight bluish tinge is preferred. The addition of the slight bluish tinge may be accomplished by any process which is known in the art including the machine blending of color concentrate prior to extrusion and the melt extrusion of blue colorants that has been pre-blended at the desired blend ratio. Colored pigments that can resist extrusion temperatures greater than 320° C. are preferred, as temperatures greater than 320° C. are necessary for coextrusion of the skin layer. Blue colorants used in this invention may be any colorant that does not have an adverse impact on the imaging element. Preferred blue colorants include Phthalocyanine blue pigments, Cromophthal blue pigments, Irgazin blue pigments, Irgalite organic blue pigments, and pigment Blue 60.

It has been found that a very thin coating (0.2 to 1.5  $\mu\text{m}$ ) on the surface immediately below the imaging layer can be made by coextrusion and subsequent stretching in the width and length direction. It has been found that this layer is, by nature, extremely accurate in thickness and can be used to provide all the color corrections which are usually distributed throughout the thickness of the sheet between the image receiving layer and the base. This topmost layer is so efficient that the total colorants needed to provide a correction are less than one-half the amount needed if the colorants are dispersed throughout thickness. Colorants are often the cause of spot defects due to clumps and poor dispersions. Spot defects, which decrease the commercial value of images, are improved with this invention because less colorant is used, and high quality filtration to clean up the colored layer is much more feasible since the total volume of polymer with colorant is only typically 2 to 10 percent of the total polymer between the transparent base and the image receiving layers.

While the addition of  $\text{TiO}_2$  in the thin skin layer of this invention does not significantly contribute to the optical performance of the sheet, it can cause numerous manufacturing problems such as extrusion die lines and spots. The skin layer substantially free of  $\text{TiO}_2$  is preferred.  $\text{TiO}_2$  added to a layer between 0.20 and 1.5  $\mu\text{m}$  does not substantially improve the optical properties of the support, will add cost to the design, and will cause objectionable pigment lines in the extrusion process.

Addenda may be added to the biaxially oriented sheet of this invention so that when the biaxially oriented sheet is viewed from a surface, the imaging element emits light in the visible spectrum when exposed to ultraviolet radiation. Emission of light in the visible spectrum allows for the support to have a desired background color in the presence of ultraviolet energy. This is particularly useful when images are viewed outside, as sunlight contains ultraviolet energy and may be used to optimize image quality for consumer and commercial applications.

Addenda known in the art to emit visible light in the blue spectrum are preferred. Consumers generally prefer a slight blue tint to white defined as a negative  $b^*$  compared to a white white defined as a  $b^*$  within one  $b^*$  unit of zero.  $b^*$  is the measure of yellow/blue in CIE space. A positive  $b^*$  indicates yellow, while a negative  $b^*$  indicates blue. The addition of addenda that emits in the blue spectrum allows for tinting the support without the addition of colorants which would decrease the whiteness of the image. The preferred emission is between 1 and 5 delta  $b^*$  units. Delta  $b^*$  is defined as the  $b^*$  difference measured when a sample is illuminated ultraviolet light source and a light source without any significant ultraviolet energy. Delta  $b^*$  is the preferred measure to determine the net effect of adding an optical brightener to the top biaxially oriented sheet of this invention. Emissions less than 1  $b^*$  unit cannot be noticed by most customers; therefore, is it not cost effective to add that amount of optical brightener to the biaxially oriented sheet. An emission greater than 5  $b^*$  units would interfere with the color balance of the prints making the whites appear too blue for most consumers.

The preferred addenda of this invention is an optical brightener. An optical brightener is colorless, fluorescent, organic compound that absorbs ultraviolet light and emits it as visible blue light. Examples include but are not limited to derivatives of 4,4'-diaminostilbene-2,2'-disulfonic acid, coumarin derivatives such as 4-methyl-7-diethylaminocoumarin, 1-4-Bis (O-Cyanostyryl) Benzol, and 2-Amino-4-Methyl Phenol.

The optical brightener may be added to any layer in the multilayer coextruded biaxially oriented polyolefin sheet. The preferred location is adjacent to or in the top surface layer of said sheet. This allows for the efficient concentration of optical brightener which results in less optical brightener being used when compared to traditional imaging supports. When the desired weight % loading of the optical brightener begins to approach the concentration at which the optical brightener migrates to the surface of the support forming crystals in the imaging layer, the addition of optical brightener into the layer adjacent to the top layer is preferred. When optical brightener migration is a concern as with imaging systems, the preferred exposed layer comprises polyethylene. In this case, the migration from the layer adjacent to the exposed layer is significantly reduced allowing for much higher optical brightener levels to be used to optimize image quality. Locating the optical brightener in the layer adjacent to the exposed layer allows for a less expensive optical brightener to be used as the exposed layer,

which is substantially free of optical brightener, and prevents significant migration of the optical brightener. Another preferred method to reduce unwanted optical brightener migration is to use polypropylene for the layer adjacent to the exposed surface. Since optical brightener is more soluble in polypropylene than polyethylene, the optical brightener is less likely to migrate from polypropylene.

A biaxially oriented sheet of this invention which has a microvoided core is preferred. The microvoided core adds opacity and whiteness to the imaging support further improving imaging quality. Combining the image quality advantages of a microvoided core with a material, which absorbs ultraviolet energy and emits light in the visible spectrum, allows for the unique optimization of image quality as the image support can have a tint when exposed to ultraviolet energy, yet retain excellent whiteness when the image is viewed using lighting that does not contain significant amounts of ultraviolet energy such as indoor lighting. The preferred number of voids in the vertical direction at substantially every point is greater than six. The number of voids in the vertical direction is the number of polymer/gas interfaces present in the voided layer. The voided layer functions as an opaque layer because of the index of refraction changes between polymer/gas interfaces. Greater than 6 voids is preferred because at 4 voids or less, little improvement in the opacity of the film is observed and, thus, does not justify the added expense to void the biaxially oriented sheet of this invention.

The microvoided core of the biaxially oriented sheet of this invention also increase the opacity of the image element without the use of  $TiO_2$  or other white pigments. During the printing process in which an image is formed in the image layers, simultaneous printing of imaging layers of the top and bottom sides is preferred to reduce printing time and increase image density. The voided layer, while providing opacity, also allows for the transmission of light.

The biaxially oriented sheet may also contain pigments which are known to improve the imaging responses such as whiteness or sharpness. Titanium dioxide is used in this invention to improve image sharpness. The  $TiO_2$  used may be either anatase or rutile type. In the case of optical properties, rutile is the preferred because of the unique particle size and geometry. Further, both anatase and rutile  $TiO_2$  may be blended to improve both whiteness and sharpness. Examples of  $TiO_2$  that are acceptable for an imaging system are DuPont Chemical Co. R101 rutile  $TiO_2$  and DuPont Chemical Co. R104 rutile  $TiO_2$ . Other pigments to improve imaging responses may also be used in this invention such as barium sulfate, clay, or calcium carbonate.

The preferred amount of  $TiO_2$  added to the biaxially oriented sheet of this invention is between 6 and 24% by weight. Below 4%  $TiO_2$ , the required reflection density of the biaxially oriented sheet is difficult to obtain. Above 28%, the desired transmission characteristics are difficult to obtain. Further, above 28%  $TiO_2$ , manufacturing efficiency declines because of  $TiO_2$  plate out on the screw, die manifold, and die lips.

For a display material to function both as a reflective display and a backlit transmission display material, the support must function as an acceptable reflective support and allow enough light to be transmitted so that support can also function as a transmission material. Further, transmission and reflection properties must be managed so that the imaging display material can be simultaneously printed on the top side and bottom sides. Due to the nature of transmission viewing materials with incorporated diffusers, (the fact that the materials are captured or suspended in a viewing

box which contains an illumination source and an air interface between the illumination source and the the display material) more transmissiviness of the display material can be tolerated and still appear sufficiently opaque in the reflection mode, while allowing for maximum transmission when used in a back lit mode.

The preferred spectral transmission of the biaxially oriented polyolefin sheet of this invention is between 35% and 90%. Spectral transmission is the amount of light energy that is transmitted through a material. For an imaging element, spectral transmission is the ratio of the transmitted power to the incident power and is expressed as a percentage as follows:  $T_{RGB}=10^{-D}*100$  where D is the average of the red, green, and blue Status A transmission density response measured by an X-Rite model 310 (or comparable) photographic transmission densitometer. The higher the transmission, the less opaque the material. Since the display material of this invention functions as both a reflective image and a transmission image, the percent transmission of the biaxially oriented sheet must be balanced to provide an acceptable reflection and transmission image. The preferred spectral transmission of the biaxially oriented polyolefin sheet of this invention is between 35% and 90% because a percent transmission of the biaxially oriented sheet less than 30%, while producing an acceptable reflection image, does not allow sufficient light to be transmitted to produce an acceptable image. A percent transmission of the biaxially oriented sheet greater than 90% is unacceptable for a quality reflection image as not enough light is reflected back to the observer's eye.

A reflection density less than 65% for the biaxially oriented sheet of this invention is preferred. Reflection density is the amount of light energy reflecting from the image to an observer's eye. Reflection density is measured by 0°/45° geometry Status A red/green/blue response using an X-Rite model 310 (or comparable) photographic transmission densitometer. A sufficient amount of reflective light energy is required to give the perception of image quality. A reflection density less than 70% is unacceptable for a reflective display material and does not match the quality of prior art reflective display materials. The most preferred reflection density for the biaxially oriented sheets of this invention is between 58% and 62%. This range allows for optimization of transmission and reflection properties to create a display material that may be used for both a reflective and transmission display material.

The coextrusion, quenching, orienting, and heat setting of these composite sheets may be effected by any process which is known in the art for producing oriented sheet, such as by a flat sheet process or a bubble or tubular process. The flat sheet process involves extruding the blend through a slit die and rapidly quenching the extruded web upon a chilled casting drum so that the core matrix polymer component of the sheet and the skin component(s) are quenched below their glass solidification temperature. The quenched sheet is then biaxially oriented by stretching in mutually perpendicular directions at a temperature above the glass transition temperature, below the melting temperature of the matrix polymers. The sheet may be stretched in one direction and then in a second direction or may be simultaneously stretched in both directions. A stretching ratio, defined as the final length divided by the original length for sum of the machine and cross directions, of at least 10 to 1 is preferred. After the sheet has been stretched, it is heat set by heating to a temperature sufficient to crystallize or anneal the polymers, while restraining to some degree the sheet against retraction in both directions of stretching.

The composite biaxially oriented polyolefin sheet, while described as having preferably at least three layers of a core and a skin layer on each side, may also be provided with additional layers that may serve to change the properties of the biaxially oriented sheet. Biaxially oriented sheets could be formed with surface layers that would provide an improved adhesion, or look to the support and imaging element. The biaxially oriented extrusion could be carried out with as many as 10 layers if desired to achieve some particular desired property.

These composite biaxially oriented polyolefin sheets may be coated or treated after the coextrusion and orienting process or between casting and full orientation with any number of coatings which may be used to improve the properties of the sheets including printability, to provide a vapor barrier, to make them heat sealable, or to improve the adhesion to the support or to the imaging layers. Examples of this would be acrylic coatings for printability, coating polyvinylidene chloride for heat seal properties. Further examples include flame, plasma, or corona discharge treatment to improve printability or adhesion.

By having at least one nonvoided skin on the microvoided core, the tensile strength of the sheet is increased and makes it more manufacturable. It allows the sheets to be made at wider widths and higher draw ratios than when sheets are made with all layers voided. Coextruding the layers further simplifies the manufacturing process.

The structure of a preferred biaxially oriented sheet where the exposed surface (top) layer is adjacent to the imaging layer is as follows:

- Polyethylene skin with blue pigments
- Polypropylene with  $TiO_2$  and optical brightener
- Polypropylene microvoided layer
- Polypropylene bottom skin layer

The support to which the microvoided, biaxially oriented sheets of this invention are laminated may be any material with the desired transmission and stiffness properties. Imaging elements of the invention can be prepared on any suitable transparent quality support including polystyrene, ceramics, synthetic high molecular weight sheet materials such as polyalkyl acrylates or methacrylates, polystyrene, polyamides such as nylon, sheets of semisynthetic high molecular weight materials such as cellulose nitrate, cellulose acetate butyrate, and the like; homo and copolymers of vinyl chloride, poly(vinylacetal), polycarbonates, homo and copolymers of olefins such as polyethylene and polypropylene, and the like.

Polyester sheets are particularly advantageous because they provide excellent strength and dimensional stability. Such polyester sheets are well known, widely used, and typically prepared from high molecular weight polyesters prepared by condensing a dihydric alcohol with a dibasic saturated fatty acid or derivative thereof.

Suitable dihydric alcohols for use in preparing such polyesters are well known in the art and include any glycol wherein the hydroxyl groups are on the terminal carbon atom and contain from 2 to 12 carbon atoms such as, for example, ethylene glycol, propylene glycol, trimethylene glycol, hexamethylene glycol, decamethylene glycol, dodecamethylene glycol, 1,4-cyclohexane, dimethanol, and the like.

Suitable dibasic acids useful for the preparation of polyesters include those containing from 2 to 16 carbon atoms such as adipic acid, sebacic acid, isophthalic acid, terephthalic acid, and the like. Alkyl esters of acids such as those listed above can also be employed. Other alcohols and acids, as well as polyesters prepared therefrom and the preparation

of the polyesters, are described in U.S. Pat. Nos. 2,720,503 and 2,901,466. Polyethylene terephthalate is preferred because it has the desired transmission and mechanical properties for a display support.

Polyester support stiffness can range from about 15 millinewtons to 100 millinewtons. The preferred stiffness is between 20 and 100 millinewtons. Polyester stiffness less than 15 millinewtons does not provide the required stiffness for display materials in that they will be difficult to handle and do not lay flat for optimum viewing. Polyester stiffness greater than 100 millinewtons begins to exceed the stiffness limit for processing equipment and has no performance benefit for the display materials.

Generally polyester films supports are prepared by melt extruding the polyester through a slit die, quenching to the amorphous state, orienting by machine and cross direction stretching, and heat setting under dimensional restraint. The polyester film can also be subjected to a heat relaxation treatment to improve dimensional stability and surface smoothness.

The polyester film will typically contain a subbing, undercoat, or primer layer on both sides of the polyester film. Subbing layers used to promote adhesion of coating compositions to the support are well known in the art and any such material can be employed. Some useful compositions for this purpose include interpolymers of vinylidene chloride such as vinylidene chloride/methyl acrylate/itaconic acid terpolymers or vinylidene chloride/acrylonitrile/acrylic acid terpolymers, and the like. These and other suitable compositions are described, for example, in U.S. Pat. Nos. 2,627,088; 2,698,240; 2,943,937; 3,143,421; 3,201,249; 3,271,178; 3,443,950; and 3,501,301. A polymeric subbing layer may be overcoated with a second subbing layer comprised of gelatin, typically referred to as gel sub.

A transparent polymer base free of  $TiO_2$  is preferred because the  $TiO_2$  in the transparent polymer gives the reflective display materials an undesirable opalescent appearance. The  $TiO_2$  pigmented transparent polymer also is expensive because the  $TiO_2$  must be dispersed into the entire thickness, typically from 100 to 180  $\mu m$ . The  $TiO_2$  also gives the transparent polymer support a slight yellow tint which is undesirable for an imaging display material. For use as an imaging reflective display material, a transparent polymer support containing  $TiO_2$  must also be tinted blue to offset the yellow tint of the polyester causing a loss in desired whiteness and adding cost to the display material. Concentration of the white pigment in the polyolefin layer allows for efficient use of the white pigment which improves image quality and reduces the cost of the imaging support.

When using a polyester base, it is preferable to extrusion laminate the microvoided composite sheets to the polyester base using a polyolefin resin. Extrusion laminating is carried out by bringing together the biaxially oriented sheets of the invention and the polyester base with application of a melt extruded adhesive between the polyester sheets and the biaxially oriented polyolefin sheets followed by their being pressed in a nip such as between two rollers. The melt extruded adhesive may be applied to either the biaxially oriented sheets or the polyester base prior to their being brought into the nip. In a preferred form the adhesive is applied into the nip simultaneously with the biaxially oriented sheets and the polyester base. The adhesive used to adhere the biaxially oriented polyolefin sheet to the polyester base may be any suitable material that does not have a harmful effect upon the imaging element. A preferred material is metallocene catalyzed ethylene plastomers that are

melt extruded into the nip between the paper and the biaxially oriented sheet. Metallocene catalyzed ethylene plastomers are preferred because they are easily melt extruded and adhere well to biaxially oriented polyolefin sheets of this invention.

The structure of a preferred reflection/transmission display support where the imaging layers are applied to the biaxially oriented polyolefin sheet is as follows:

Biaxially oriented polyolefin sheet

Metallocene catalyzed ethylene plastomer

Polyester base

As used herein, the phrase "imaging element" is a material that utilizes nonphotographic or nonsilver halide imaging technology in the formation of images. Nonphotographic imaging methods include thermal dye transfer, ink jet, electrophotographic, electrographic, flexographic printing, or rotogravure printing. The imaging layers of this invention are preferably coated on the top and the bottom sides.

For the display material of this invention, at least one image layer located on the top side of said imaging element is suitable. Applying the imaging layer to either the top or bottom is suitable for a day/night display material; however, it is not sufficient to create a day/night display material that is optimum for both a reflective display and a transmission display. For the display material of this invention, at least one image layer on both the top and bottom of the imaging support of this invention is preferred. Applying an image layer to both the top and bottom of the support allows for the display material to have the required density for reflective viewing and for transmission viewing of the image. An imaging layer on one side with double density, while having the required density for transmission, would appear too dark in reflection. Thus, an image formed on both sides is preferred. This dual "day/night" display material has significant commercial value in that the day/night display material can be used for both reflective viewing and transmission viewing. Prior art display materials were optimized for either transmission viewing or reflective viewing, but not both simultaneously.

The thermal dye image-receiving layer of the receiving elements of the invention may comprise, for example, a polycarbonate, a polyurethane, a polyester, polyvinyl chloride, poly(styrene-co-acrylonitrile), poly(caprolactone), or mixtures thereof. The dye image-receiving layer may be present in any amount which is effective for the intended purpose. In general, good results have been obtained at a concentration of from about 1 to about 10 g/m<sup>2</sup>. An overcoat layer may be further coated over the dye-receiving layer, such as described in U.S. Pat. No. 4,775,657 of Harrison et al.

Dye-donor elements that are used with the dye-receiving element of the invention conventionally comprise a support having thereon a dye containing layer. Any dye can be used in the dye-donor employed in the invention provided it is transferable to the dye-receiving layer by the action of heat. Especially good results have been obtained with sublimable dyes. Dye donors applicable for use in the present invention are described, e.g., in U.S. Pat. Nos. 4,916,112; 4,927,803; and 5,023,228.

As noted above, dye-donor elements are used to form a dye transfer image. Such a process comprises image-wise-heating a dye-donor element and transferring a dye image to a dye-receiving element as described above to form the dye transfer image.

In a preferred embodiment of the thermal dye transfer method of printing, a dye donor element is employed which compromises a poly-(ethylene terephthalate) support coated

with sequential repeating areas of cyan, magenta, and yellow dye, and the dye transfer steps are sequentially performed for each color to obtain a three-color dye transfer image. Of course, when the process is only performed for a single color, then a monochrome dye transfer image is obtained.

Thermal printing heads which can be used to transfer dye from dye-donor elements to receiving elements of the invention are available commercially. There can be employed, for example, a Fujitsu Thermal Head (FTP-040 MCS001), a 10 TDK Thermal Head F415 HH7-1089, or a Rohm Thermal Head KE 2008-F3. Alternatively, other known sources of energy for thermal dye transfer may be used, such as lasers as described in, for example, G.B. 2,083,726A.

A thermal dye transfer assemblage comprises (a) a dye-donor element, and (b) a dye-receiving element as described above, the dye-receiving element being in a superposed relationship with the dye-donor element so that the dye layer of the donor element is in contact with the dye image-receiving layer of the receiving element.

When a three-color image is to be obtained, the above assemblage is formed on three occasions during the time when heat is applied by the thermal printing head. After the first dye is transferred, the elements are peeled apart. A second dye-donor element (or another area of the donor element with a different dye area) is then brought in register with the dye-receiving element and the process repeated. The third color is obtained in the same manner.

The electrographic and electrophotographic processes and their individual steps have been well described in detail in many books and publications. The processes incorporate the basic steps of creating an electrostatic image, developing that image with charged, colored particles (toner), optionally transferring the resulting developed image to a secondary substrate, and fixing the image to the substrate. There are numerous variations in these processes and basic steps; the use of liquid toners in place of dry toners is simply one of those variations.

The first basic step, creation of an electrostatic image, can be accomplished by a variety of methods. The electrophotographic process of copiers uses imagewise photo discharge, through analog or digital exposure, of a uniformly charged photoconductor. The photoconductor may be a single-use system, or it may be rechargeable and reimagineable, like those based on selenium or organic photoreceptors.

In one form of the electrophotographic process, copiers use imagewise photo discharge, through analog or digital exposure, of a uniformly charged photoconductor. The photoconductor may be a single-use system, or it may be 50 rechargeable and reimagineable, like those based on selenium or organic photoreceptors.

In one form of the electrophotographic process, a photo-sensitive element is permanently imaged to form areas of differential conductivity. Uniform electrostatic charging, 55 followed by differential discharge of the imaged element, creates an electrostatic image. These elements are called electrographic or xeroprinting masters because they can be repeatedly charged and developed after a single imaging exposure.

In an alternate electrographic process, electrostatic images are created iono-graphically. The latent image is created on dielectric (charge-holding) medium, either paper or film. Voltage is applied to selected metal styli or writing nibs from an array of styli spaced across the width of the medium, causing a dielectric breakdown of the air between the selected styli and the medium. Ions are created, which form the latent image on the medium.

Electrostatic images, however generated, are developed with oppositely charged toner particles. For development with liquid toners, the liquid developer is brought into direct contact with the electrostatic image. Usually a flowing liquid is employed, to ensure that sufficient toner particles are available for development. The field created by the electrostatic image causes the charged particles, suspended in a nonconductive liquid, to move by electrophoresis. The charge of the latent electrostatic image is thus neutralized by the oppositely charged particles. The theory and physics of electrophoretic development with liquid toners are well described in many books and publications.

If a reimagineable photoreceptor or an electrographic master is used, the toned image is transferred to paper (or other substrate). The paper is charged electrostatically, with the polarity chosen to cause the toner particles to transfer to the paper. Finally, the toned image is fixed to the paper. For self-fixing toners, residual liquid is removed from the paper by air-drying or heating. Upon evaporation of the solvent, these toners form a film bonded to the paper. For heat-fusible toners, thermoplastic polymers are used as part of the particle. Heating both removes residual liquid and fixes the toner to paper.

The dye receiving layer or DRL for ink jet imaging may be applied by any known methods, such as solvent coating or melt extrusion coating techniques. The DRL is coated over the tie layer or TL at a thickness ranging from 0.1–10  $\mu\text{m}$ , preferably 0.5–5  $\mu\text{m}$ . There are many known formulations which may be useful as dye receiving layers. The primary requirement is that the DRL is compatible with the inks which it will be imaged so as to yield the desirable color gamut and density. As the ink drops pass through the DRL, the dyes are retained or mordanted in the DRL, while the ink solvents pass freely through the DRL and are rapidly absorbed by the TL. Additionally, the DRL formulation is preferably coated from water, exhibits adequate adhesion to the TL, and allows for easy control of the surface gloss.

For example, Misuda et al., in U.S. Pat. Nos. 4,879,166; 5,14,730; 5,264,275; 5,104,730; 4,879,166; and Japanese Patent Nos. 1,095,091; 2,276,671; 2,276,670; 4,267,180; 5,024,335; and 5,016,517 discloses aqueous based DRL formulations comprising mixtures of pseudo-bohemite and certain water soluble resins. Light, in U.S. Pat. Nos. 4,903,040; 4,930,041; 5,084,338; 5,126,194; 5,126,195; 5,139,8667; and 5,147,717 discloses aqueous-based DRL formulations comprising mixtures of vinyl pyrrolidone polymers and certain water-dispersible and/or water-soluble polyesters, along with other polymers and addenda. Butters et al. in U.S. Pat. Nos. 4,857,386 and 5,102,717 disclose ink-absorbent resin layers comprising mixtures of vinyl pyrrolidone polymers and acrylic or methacrylic polymers. Sato, et al. in U.S. Pat. No. 5,194,317 and Higuma et al. in U.S. Pat. No. 5,059,983 disclose aqueous-coatable DRL formulations based on poly (vinyl alcohol). Iqbal in U.S. Pat. No. 5,208,092 discloses water-based ink receiver layer or IRL formulations comprising vinyl copolymers which are subsequently cross-linked. In addition to these examples, there may be other known or contemplated DRL formulations which are consistent with the aforementioned primary and secondary requirements of the DRL, all of which fall under the spirit and scope of the current invention.

The preferred DRL is a 0.1–10  $\mu\text{m}$  DRL which is coated as an aqueous dispersion of 5 parts alumoxane and 5 parts poly (vinyl pyrrolidone). The DRL may also contain varying levels and sizes of matting agents for the purpose of controlling gloss, friction, and/or fingerprint resistance, surfactants to enhance surface uniformity and to adjust the surface

tension of the dried coating, mordanting agents, antioxidants, UV absorbing compounds, light stabilizers, and the like.

Although the ink-receiving elements as described above can be successfully used to achieve the objectives of the present invention, it may be desirable to overcoat the DRL for the purpose of enhancing the durability of the imaged element. Such overcoats may be applied to the DRL either before or after the element is imaged. For example, the DRL can be overcoated with an ink-permeable layer through which inks freely pass. Layers of this type are described in U.S. Pat. Nos. 4,686,118; 5,027,131; and 5,102,717 in European Patent Specification 0 524 626, and also in pending U.S. patent applications based on DN 71302. Alternatively, an overcoat may be added after the element is imaged. Any of the known laminating films and equipment may be used for this purpose. The inks used in the aforementioned imaging process are well known, and the ink formulations are often closely tied to the specific processes, i.e., continuous, piezoelectric, or thermal. Therefore, depending on the specific ink process, the inks may contain widely differing amounts and combinations of solvents, colorants, preservatives, surfactants, humectants, and the like. Inks preferred for use in combination with the image recording elements of the present invention are water-based, such as those currently sold for use in the Hewlett-Packard Desk Writer 560C printer. However, it is intended that alternative embodiments of the image-recording elements as described above, which may be formulated for use with inks which are specific to a given ink-recording process or to a given commercial vendor, fall within the scope of the present invention.

Printing generally accomplished by Flexographic or Rotogravure. Flexography is an offset letterpress technique where the printing plates are made from rubber or photo-polymer. The printing is accomplished by the transfer of the ink from the raised surface of the printing plate to the support of this invention. The Rotogravure method of printing uses a print cylinder with thousands of tiny cells which are below the surface of the printing cylinder. The ink is transferred from the cells when the print cylinder is brought into contact with the web at the impression roll.

Suitable inks for this invention include solvent based inks, water based inks, and radiation cured inks. Examples of solvent based inks include nitrocellulose maleic, nitrocellulose polyamide, nitrocellulose acrylic, nitrocellulose urethane, chlorinated rubber, vinyl, acrylic, alcohol soluble acrylic, cellulose acetate acrylic styrene, and other synthetic polymers. Examples of water based inks include acrylic emulsion, maleic resin dispersion, styrene maleic anhydride resins, and other synthetic polymers. Examples of radiation cured inks include ultraviolet and electron beam cure inks.

When the support of this invention is printed with Flexographic or Rotogravure inks, an ink adhesion coating may be required to allow for efficient printing of the support. The top layer of the biaxially oriented sheet may be coated with any materials known in the art to improve ink adhesion to biaxially oriented polyolefin sheets of this invention. Examples include acrylic coatings and polyvinyl alcohol coatings. Surface treatments to the biaxially oriented sheets of this invention may also be used to improve ink adhesion. Examples include corona and flame treatment.

The following examples illustrate the practice of this invention. They are not intended to be exhaustive of all possible variations of the invention. Parts and percentages are by weight unless otherwise indicated.

## EXAMPLES

### Example 1

In this example, a transparent polyester base materials was laminated with a microvoided biaxially oriented poly-

olefin sheet containing blue tints, optical brightener, and  $TiO_2$ . The support structure in this example was coated with an ink jet printing dye receiver layer on both sides of the support. This example will show the desirable increase in stiffness when the biaxially oriented sheet is laminated to the polyester sheet. Further, this example will also show that a quality display image can be produced that can function as both a transmission display material and a reflection display material. The following laminated imaging display material (invention) was prepared by extrusion laminating the following biaxially oriented polymer sheet to top side of a photographic grade polyester base:

Top Sheet

A composite sheet consisting of 5 layers identified as L1, L2, L3, L4, and L5. L1 is the thin colored layer on the outside (top) of the package to which the ink jet dye receiving layer was coated. L2 is the layer to which optical brightener and  $TiO_2$  was added. The optical brightener used was Hostalux KS manufactured by Ciba-Geigy. Rutile  $TiO_2$  was added to the L2 at 12% by weight of base polymer. The  $TiO_2$  type was DuPont R104 (a 0.22  $\mu m$  particle size  $TiO_2$ ). Table 1 below lists the characteristics of the layers of the biaxially oriented sheet used in this example.

TABLE 1

| Layer | Material                            | Thickness, $\mu m$ |
|-------|-------------------------------------|--------------------|
| L1    | LD Polyethylene + color concentrate | 0.75               |
| L2    | Polypropylene + $TiO_2$ + OB        | 4.32               |
| L3    | Voided Polypropylene                | 24.9               |
| L4    | Polypropylene                       | 4.32               |
| L5    | Polypropylene                       | 0.762              |
| L6    | LD Polyethylene                     | 11.4               |

Photographic Grade Polyester Base

A polyethylene terephthalate sheet base 110  $\mu m$  thick that was transparent and gelatin coated on both sides of the base and dried. The polyethylene terephthalate base had a stiffness of 30 millinewtons in the machine direction and 40 millinewtons in the cross direction.

The top sheet used in this example was coextruded and biaxially oriented. The top sheet was melt extrusion laminated to the polyester sheet base using an metallocene catalyzed ethylene plastomer (SLP 9088) manufactured by Exxon Chemical Corp. The metallocene catalyzed ethylene plastomer had a density of 0.900 g/cc and a melt index of 14.0.

The L3 layer for the biaxially oriented sheet is microvoided and further described in Table 2 where the refractive index and geometrical thickness is shown for measurements made along a single slice through the L3 layer. The measurements do not imply continuous layers, a slice along another location would yield different but approximately the same thickness. The areas with a refractive index of 1.0 are voids that are filled with air and the remaining layers are polypropylene.

TABLE 2

| Sublayer of L3 | Refractive Index | Thickness, $\mu m$ |
|----------------|------------------|--------------------|
| 1              | 1.49             | 2.54               |
| 2              | 1                | 1.527              |
| 3              | 1.49             | 2.79               |
| 4              | 1                | 1.016              |
| 5              | 1.49             | 1.778              |
| 6              | 1                | 1.016              |
| 7              | 1.49             | 2.286              |

TABLE 2-continued

| Sublayer of L3 | Refractive Index | Thickness, $\mu m$ |
|----------------|------------------|--------------------|
| 8              | 1                | 1.016              |
| 9              | 1.49             | 2.032              |
| 10             | 1                | 0.762              |
| 11             | 1.49             | 2.032              |
| 12             | 1                | 1.016              |
| 13             | 1.49             | 1.778              |
| 14             | 1                | 1.016              |
| 15             | 1.49             | 2.286              |

An ink jet image receiving layer was utilized to prepare the display material of this example and was coated on the L1 polyethylene layer on the top biaxially oriented sheet and coated on the bottom gelatin layer on the transparent polyester base. The ink jet image receiving layer was coated by means of an extrusion hopper a dispersion containing 326.2 g of gelatin, 147 g of BVSME hardener, i.e., (bis (vinylsulfonylmethyl) ether 2% solution in water, 7.38 g of a dispersion containing 2.88 g of 11.5  $\mu m$  polystyrene beads, 0.18 g of Dispex(TM) (40% solution in water obtained from Allied Colloids, Inc.), and 4.32 g of water, and 3.0 g of a 20% solution in water of Surfactant 10G (nonylphenoxy polyglycidol) obtained from Olin Matheson Company. The thickness was about 5  $\mu m$  (dried thickness).

Onto this layer was coated by means of an extrusion hopper an aqueous solution containing 143.5 g of a 3% solution in water of 4.42 g of hydroxypropyl cellulose (Methocel KLV100, Dow Chemical Company), 0.075 g of vanadyl sulfate, 2-hydrate obtained from Eastman Kodak Company, 0.075 g of a 20% solution in water of Surfactant 10G (nonylphenoxy polyglycidol) obtained from Olin Matheson Company, and 145.4 g of water; and 0.45 g of a 20% solution in water of Surfactant 10G (nonylphenoxy polyglycidol) obtained from Olin Matheson Company and 79.5 g of water to form an ink-receiving layer about 2  $\mu m$  in thickness (dry thickness).

The structure of the invention in this example was as follows:

Ink jet receiving layer  
Biaxially oriented, microvoided polyolefin sheet  
Metallocene ethylene plastomer  
Gelatin sub coating  
Transparent polyester base  
Gelatin sub coating  
Ink jet receiving layer

The bending stiffness of the polyester base and the laminated display material support was measured by using the Lorentzen and Wettre stiffness tester, Model 16D. The output from this instrument is force, in millinewtons, required to bend the cantilevered, unclasped end of a sample 20 mm long and 38.1 mm wide at an angle of 15 degrees from the unloaded position. In this test the stiffness in both the machine direction and cross direction of the polyester base was compared to the stiffness of the base laminated with the top biaxially oriented sheet of this example. The results are presented in Table 3.

TABLE 3

|                   | Machine Direction Stiffness (millinewtons) | Cross Direction Stiffness (millinewtons) |
|-------------------|--------------------------------------------|------------------------------------------|
| Before Lamination | 33                                         | 23                                       |
| After Lamination  | 87                                         | 80                                       |

The data above in Table 3 show the significant increase in stiffness of the polyester base after lamination with a biaxially oriented polymer sheet. This result is significant in that prior art materials, in order to provide the necessary stiffness, used polyester bases that were much thicker (between 150 and 256  $\mu\text{m}$ ) compared to the 110  $\mu\text{m}$  polyester base used in this example. At equivalent stiffness, the significant increase in stiffness after lamination allows for a thinner polyester base to be used compared to prior art materials, thus reducing the cost of the display support. Further, a reduction in display material thickness allows for a reduction in material handling costs, as rolls of thinner material weigh less and are smaller in roll diameter.

The display support was measured for status A density using an X-Rite Model 310 photographic densitometer. Spectral transmission is calculated from the Status A density readings and is the ratio of the transmitted power to the incident power and is expressed as a percentage as follows:  $T_{RGB}=10^{-D} \cdot 100$  where D is the average of the red, green, and blue Status A transmission density response. The display material were also measured for  $L^*$ ,  $a^*$ , and  $b^*$  using a Spectrogard spectrophotometer, CIE system, using illuminant D6500. In the transmission mode, a qualitative assessment was made as to the amount of illuminating backlighting show through. A substantial amount of show through would be considered undesirable, as the nonfluorescent light sources could interfere with the image quality. The display material of this example was printed with various test images on a Hewlett Packard DeskJet 870 Cxi ink jet printer. The performance data for invention is listed in Table 4 below.

TABLE 4

| Measure                            | Invention measured in Transmission |
|------------------------------------|------------------------------------|
| % Transmission                     | 38%                                |
| CIE D6500 $L^*$                    | 64.19                              |
| CIE D6500 $a^*$                    | -0.29                              |
| CIE D6500 $b^*$                    | 0.67                               |
| Illuminating Backlight Showthrough | None                               |

The reflection/transmission display support coated on the top and bottom sides with the ink jet ink receiving layer of this example exhibits all the properties needed for an imaging display material that can function as both a reflective and transmission display material. Further the imaging reflection/transmission display material of this example has many advantages. The nonvoided layers have levels of  $\text{TiO}_2$  and colorants adjusted to provide an improved minimum density position as the invention was able to overcome the native yellowness that is common with gelatin based ink or dye receiving layers. The density minimum  $b^*$  for the invention was 0.67 which is substantially neutral and preferred over a yellow density minimum. In the transmission

mode, the illuminating backlights did not show through, indicating the invention was able to diffuse the illuminating backlight and allow enough light to be transmitted to provide a quality image.

- 5 The 38% transmission for the invention provides an acceptable reflection image and allow enough light through the support to be an acceptable transmission image. A display material that functions as both transmission materials and reflective materials has significant commercial value, as the quality of the display image is robust to lighting factors such as the amount of sunlight or the intensity of the illuminating light source. Since the display material can function in both transmission and reflection, inventories can be consolidated in manufacturing and at the point of use. 10 15 Further, concentration of the tint materials and the white pigments in the biaxially oriented sheet allows for manufacturing efficiency and lower material utilization resulting in a low cost display material. The  $a^*$  and  $L^*$  for the invention are consistent with high quality reflective and transmission display materials. Finally the invention would be low in cost over prior art materials display materials as a 4.0 mil polyester base was used in the invention compared to a 8.7 mil polyester for prior art display materials.

Finally, because of the duplitzed ink jet dye receiving layer, the invention could be imaged on both sides providing the ink density for a reflective image and when backlit, providing the required ink density for a high quality transmission image. Because digital ink jet printing technology was utilized to form the images, the images was printed in 12 minutes compared to a typical time to image of several days for photographic transmission display materials.

The invention has been described in detail with particular reference to preferred embodiments thereof, but it will be understood that variations and modifications can be effected within the spirit and scope of the invention.

#### What is claimed is:

1. An imaging element comprising a transparent polymer sheet, at least one layer of biaxially oriented polyolefin sheet and at least one image receiving layer wherein said polymer sheet has a stiffness of between 20 and 100 millinewtons, and said biaxially oriented polyolefin sheet has a spectral transmission of between 35% and 90% and a reflection density of between 15% and 65% wherein said at least one image receiving layer comprises at least one ink jet receiving layer.
2. The imaging element of claim 1 wherein said biaxially oriented polyolefin sheet contains white pigment.
3. The imaging element of claim 1 wherein said biaxially oriented polyolefin sheet further comprises microvoids.
4. The imaging element of claim 3 wherein said microvoids comprise at least one layer of said biaxially oriented polyolefin sheet and have at least 6 voids in the vertical direction at substantially every point of the biaxially oriented polyolefin sheet.
5. The imaging element of claim 1 wherein said biaxially oriented polyolefin sheet has an integral layer of polyethylene on the top of said sheet.
6. The imaging element of claim 1 wherein said element comprises between 6 and 24 weight percent of titanium dioxide.
7. The imaging element of claim 6 wherein said titanium dioxide is a layer above said biaxially oriented polyolefin sheet.
8. The imaging element of claim 1 wherein said element has a reflection density of between 58 and 62%.
9. The imaging element of claim 1 wherein said transparent polymer sheet is substantially free of pigment.

**10.** The imaging element of claim **1** wherein said at least one image receiving layer comprises at least one image receiving layer located on the top side of said biaxially oriented polyolefin sheet and said biaxially oriented polyolefin sheet is located above said transparent polymer sheet.

**11.** The imaging element of claim **10** further comprising at least one image receiving layer located on the opposite side of said transparent polymer sheet from the biaxially oriented polyolefin sheet.

**12.** The imaging element of claim **1** wherein said element comprises at least one printing ink receiving layer.

**13.** The imaging element of claim **1** wherein said element comprises an imaging receiving layer on both sides of said imaging element.

**14.** The image receiving member of claim **1** wherein said at least one image receiving member is located adjacent said transparent polymer sheet.

**15.** The imaging element of claim **14** wherein said element has a reflection density of between 58 and 62%.

**16.** An imaging element comprising a transparent polymer sheet, at least one layer of biaxially oriented polyolefin sheet and at least one image receiving layer wherein said polymer sheet has a stiffness of between 20 and 100 millinewtons, and said biaxially oriented polyolefin sheet has a spectral transmission of between 35% and 90% and a reflection density of between 15% and 65% wherein said at least one image receiving layer comprises at least one electrophotographic receiving layer.

**17.** The imaging element of claim **16** wherein said biaxially oriented polyolefin sheet contains white pigment.

**18.** The imaging element of claim **16** wherein said biaxially oriented polyolefin sheet further comprises microvoids.

**19.** The imaging element of claim **18** wherein said microvoids comprise at least one layer of said biaxially oriented polyolefin sheet and have at least 6 voids in the vertical direction at substantially every point of the biaxially oriented polyolefin sheet.

**20.** The imaging element of claim **16** wherein said biaxially oriented polyolefin sheet has an integral layer of polyethylene on the top of said sheet.

**21.** The imaging element of claim **16** wherein said element comprises between 6 and 24 weight percent of titanium dioxide.

**22.** The imaging element of claim **21** wherein said titanium dioxide is a layer above said biaxially oriented polyolefin sheet.

**23.** The imaging element of claim **16** wherein said transparent polymer sheet is substantially free of pigment.

**24.** The imaging element of claim **16** wherein said at least one image receiving layer comprises at least one image receiving layer located on the top side of said biaxially oriented polyolefin sheet and said biaxially oriented polyolefin sheet is located above said transparent polymer sheet.

**25.** The imaging element of claim **24** further comprising at least one image layer located on the opposite side of said transparent polymer sheet from the biaxially oriented polyolefin sheet.

**26.** The imaging element of claim **16** wherein said element comprises an image receiving layer on both sides of said imaging element.

**27.** An imaging element comprising a transparent polymer sheet, at least one layer of biaxially oriented polyolefin sheet and at least one image receiving layer wherein said polymer sheet has a stiffness of between 20 and 100 millinewtons, and said biaxially oriented polyolefin sheet has a spectral transmission of between 35% and 90% and a reflection density of between 15% and 65% wherein said at least one image receiving layer comprises at least one printing ink receiving layer.

**28.** The imaging element of claim **27** wherein said biaxially oriented polyolefin sheet contains white pigment.

**29.** The imaging element of claim **27** wherein said biaxially oriented polyolefin sheet further comprises microvoids.

**30.** The imaging element of claim **29** wherein said microvoids comprise at least one layer of said biaxially oriented polyolefin sheet and have at least 6 voids in the vertical direction at substantially every point of the biaxially oriented polyolefin sheet.

**31.** The imaging element of claim **27** wherein said biaxially oriented polyolefin sheet has an integral layer of polyethylene on the top of said sheet.

**32.** The imaging element of claim **27** wherein said element comprises between 6 and 24 weight percent of titanium dioxide.

**33.** The imaging element of claim **32** wherein said titanium dioxide is a layer above said biaxially oriented polyolefin sheet.

**34.** The imaging element of claim **27** wherein said element has a reflection density of between 58 and 62%.

**35.** The imaging element of claim **27** wherein said transparent polymer sheet is substantially free of pigment.

**36.** The imaging element of claim **27** wherein said at least one image receiving layer comprises at least one image receiving layer located on the top side of said biaxially oriented polyolefin sheet and said biaxially oriented polyolefin sheet is located above said transparent polymer sheet.

**37.** The imaging element of claim **36** further comprising at least one image layer located on the opposite side of said transparent polymer sheet from the biaxially oriented polyolefin sheet.

**38.** The imaging element of claim **36** wherein said element comprises an image receiving layer on both sides of said imaging element.